

Nov. 20, 1956

J. J. COLEMAN ET AL

2,771,380

METHOD OF PLATING COPPER PARTICLES WITH SILVER

Filed Aug. 2, 1954



INVENTORS:

and Joseph J. Coleman  
Emil M. Dittman  
By: Jones, Darby & Robertson Atty's.

1

2,771,380

## METHOD OF PLATING COPPER PARTICLES WITH SILVER

Joseph J. Coleman and Emil M. Dittman, Freeport, Ill.,  
assignors to Burgess Battery Company, Freeport, Ill.,  
a corporation of Delaware

Application August 2, 1954, Serial No. 447,409

5

10

8 Claims. (Cl. 117—227)

This invention relates to a method for plating copper particles with silver, and particularly to an immersion type of method, as distinguished from an electrolytic method, of plating copper particles with silver.

The immersion plating of copper with silver is accomplished by immersing the articles to be plated in an aqueous cyanide silver plating bath, and in the plating of copper particles there is a tendency for the particles to agglomerate or adhere together in the form of small masses or pellets. This has two undesirable effects, the first being that the agglomeration itself is objectionable, and the second being that the copper particles are incompletely coated or plated with silver.

It is an object of the invention to provide a method for the immersion plating of copper particles with silver in which the objectionable agglomeration is avoided and complete and continuous coatings or plates of silver are obtained upon the individual copper particles.

The process of the invention is indicated by the flow sheet shown in the drawing.

The method of the invention is applicable to copper particles of any form including flakes. Such particles are susceptible to agglomeration and the method of the invention is effective in avoiding agglomeration of copper particles of any form including flakes during plating thereof with silver. The method has been used with success with particles which range in size from about one millimeter to a few microns in their maximum dimension. Small silver coated copper particles of this character find usefulness as an ingredient in electrically conductive compositions, as for example, in admixture with a binder or vehicle to form a conductive composition or paint.

In accordance with the invention, the copper particles are immersed in the aqueous silver plating bath in the presence of a medium or agent which maintains the copper particles in separated or dispersed condition. In one procedure, the separating agent is in the form of discrete water-soluble bodies such as crystalline hydrated sodium sulfate (Glauber's salt), potassium sulfate, sodium nitrate or the like. In a preferred procedure, the copper particles are first dry mixed with the discrete bodies and the mixture is immersed in an aqueous cyanide silver plating bath. The water-soluble bodies are larger than the copper particles and the volume of said bodies is substantially greater than that of the copper particles, whereby the copper particles become attached to the surfaces of said bodies in separated or dispersed condition and not in agglomerated condition. A suitable size for the water-soluble bodies is from 0.25 inch to .0014 inch. The water-soluble bodies may be in the form of preformed pellets, or crystals produced by crystallization processes, or granules formed by the fracture of larger bodies.

As an example of the method, 30 parts by weight of flake copper is dry mixed with 400 parts of bodies of hydrated sodium sulfate,  $\text{Na}_2\text{SO}_4 \cdot 10\text{H}_2\text{O}$ , in a suitable blender or mixer until the copper particles become attached in the form of a coating of dispersed particles to

2

the surfaces of the sodium sulfate bodies. The mixture of flake copper and hydrated sodium sulfate bodies is then immersed in 800 parts of a cyanide silver plating solution, constant agitation being maintained during the immersion. The plating bath may be of conventional composition as follows, the proportions being in parts by weight:

|                     |      |
|---------------------|------|
| Silver cyanide      | 125  |
| Potassium cyanide   | 125  |
| Potassium carbonate | 25   |
| Water               | 1825 |

Agitation is continued until the sodium sulfate becomes dissolved in the plating solution, when it is discontinued and the solution is allowed to stand until the particles have settled to the bottom of the container. During the agitation and solution of the sodium sulfate, a plating of the copper particles with silver takes place by a chemical deposition of silver from the silver cyanide in the plating bath. The silver-coated particles are separated from the plating bath in any suitable manner as by decantation and are then thoroughly washed with water and dried.

It has been found that in the process which has been described the silver is deposited in the form of a complete and continuous coating or plate upon the surfaces of the individual copper particles. The individual particles are visible to the eye, thereby showing their non-agglomeration. The bright silver color of the particles is also visible to the eye, thereby showing the complete coating of the individual particles with silver. Upon analysis the particles are found to contain 12 percent by weight of silver.

To further demonstrate that complete silver coatings are produced upon the individual copper particles by the process of the invention, a conductive composition was prepared containing the particles resulting from the method which is described in the foregoing example. The particles were thoroughly mixed with molten microcrystalline wax, the proportions being 14 parts by weight of microcrystalline wax and 18 parts of particles. The composition was then cooled to room temperature with solidification of the microcrystalline wax, and was extruded under pressure into the form of a cylindrical section  $\frac{1}{8}$  inch in diameter and 6 inches long. The resistance of the section was measured and found to be less than one ohm.

For comparison purposes, similar copper particles were subjected to a plating method exactly the same as described in the foregoing example except that the hydrated sodium sulfate bodies were dispensed with. The resulting plated copper was in the form of silver-coated masses or pellets which were round or nearly round in shape. The pellets were broken open and the interiors were found to be composed of uncoated copper flakes which upon standing in the atmosphere turned dark in color. The silver-coated pellets were subjected to a mild crushing operation to separate the agglomerations into individual particles. When mixed with microcrystalline wax in the manner described in the foregoing, the resulting composition exhibits an extremely high resistance such that for practical purposes it is a non-conductor.

The superior conductivity of the composition containing the particles plated in accordance with the present invention is due to the fact that the copper particles are completely coated by silver whereas the other particles are not. Copper is subject to the acquisition in the atmosphere of a surface factor which greatly increases the contact resistance, whereas silver is substantially unaffected in this way.

Invention is claimed as follows:

1. The method of plating copper particles with silver

which comprises dry mixing said copper particles with discrete water-soluble bodies whereby said copper particles become attached to the surfaces of said water-soluble bodies, said water-soluble bodies being of a size substantially larger than that of said copper particles and the volume of the water-soluble bodies being greater than that of the copper particles and being sufficient that the copper particles are in dispersed condition on the surfaces of the water-soluble bodies, immersing said mixture in an immersion type aqueous silver plating bath, causing said water-soluble bodies to be dissolved in said plating bath, and separating the resulting silver plated copper particles from said plating bath.

2. The method of plating copper particles with silver which comprises dry mixing said copper particles with discrete water-soluble bodies whereby said copper particles become attached to the surfaces of said water-soluble bodies, said water-soluble bodies being of a size substantially larger than that of said copper particles and the volume of the water-soluble bodies being greater than that of the copper particles and being sufficient that the copper particles are in dispersed condition on the surfaces of the water-soluble bodies, immersing said mixture in an immersion type aqueous silver plating bath, and causing said water-soluble bodies to be dissolved in said plating bath.

3. The method of plating copper particles with silver which comprises dry mixing said copper particles with discrete water-soluble bodies whereby said copper particles become attached to the surfaces of said water-soluble bodies, immersing said mixture in an immersion type aqueous silver plating bath, and causing said water-soluble bodies to be dissolved in said plating bath.

4. The method of plating copper particles with silver which comprises immersing said copper particles in an immersion type aqueous silver plating bath while attached to the surfaces of undissolved water-soluble bodies of a size greater than that of said copper particles.

5. The method of plating copper particles with silver which comprises dry mixing said copper particles with discrete bodies of crystalline hydrated sodium sulfate whereby said copper particles become attached to the surfaces of said sodium sulfate bodies, said sodium sulfate bodies being of a size substantially larger than that of said copper particles and the volume of sodium sulfate bodies being greater than that of the copper particles

and being sufficient that the copper particles are in dispersed condition upon the surfaces of the sodium sulfate bodies, immersing said mixture in an immersion type aqueous silver plating bath, causing said sodium sulfate to be dissolved in said plating bath, and separating the resulting silver plated copper particles from said plating bath.

6. The method of plating copper particles with silver which comprises dry mixing said copper particles with bodies of crystalline hydrated sodium sulfate whereby said copper particles become attached to the surfaces of said sodium sulfate bodies, said sodium sulfate bodies being of a size substantially larger than that of said copper particles and the volume of sodium sulfate bodies being greater than that of the copper particles and being sufficient that the copper particles are in dispersed condition and are not agglomerated upon the surfaces of the sodium sulfate bodies, immersing said mixture in an immersion type aqueous silver plating bath and causing said sodium sulfate to be dissolved in said plating bath.

7. The method of plating copper particles with silver which comprises dry mixing said copper particles with bodies of crystalline hydrated sodium sulfate whereby said copper particles become attached to the surfaces of said sodium sulfate bodies, immersing said mixture in an immersion type aqueous silver plating bath, and causing said sodium sulfate to be dissolved in said plating bath.

8. The method as claimed in claim 4 in which the copper particles are in the form of flakes.

#### References Cited in the file of this patent

##### UNITED STATES PATENTS

|    |           |                 |       |               |
|----|-----------|-----------------|-------|---------------|
| 35 | 1,208,507 | Dalby           | ----- | Dec. 12, 1916 |
|    | 2,110,792 | Egeberg et al.  | ----- | Mar. 8, 1938  |
|    | 2,113,517 | Powell et al.   | ----- | Apr. 5, 1938  |
|    | 2,391,289 | Beaver          | ----- | Dec. 18, 1945 |
|    | 2,472,393 | Avallone et al. | ----- | June 7, 1949  |
| 40 | 2,613,179 | Wolfson et al.  | ----- | Oct. 7, 1952  |

##### FOREIGN PATENTS

|         |               |       |              |
|---------|---------------|-------|--------------|
| 396,250 | Great Britain | ----- | Aug. 3, 1933 |
|---------|---------------|-------|--------------|

##### OTHER REFERENCES

|    |                                                                                       |
|----|---------------------------------------------------------------------------------------|
| 45 | Sanigar: The Electrochemical Society, Preprint 59-33, April 27, 1931, pp. 363 to 367. |
|----|---------------------------------------------------------------------------------------|